

# UNITED STATES PATENT OFFICE.

DAVID LAMON, OF DENVER, COLORADO.

## PROCESS OF TREATING IRON AND STEEL.

1,096,006.

Specification of Letters Patent.

Patented May 5, 1914.

No Drawing.

Application filed December 20, 1910. Serial No. 598,313.

*To all whom it may concern:*

Be it known that I, DAVID LAMON, a citizen of the United States, and a resident of Denver, in the county of Denver and State of Colorado, have made certain new and useful Improvements in Processes of Treating Iron and Steel, of which the following is a specification.

My invention relates to improvements in compositions of matter for hardening and otherwise improving the physical properties of iron and steel, and it consists in the various ingredients hereinafter enumerated.

This invention is an improvement over a similar one set forth in my prior Patent #892,269, June 30, 1908. In the prior patent, just mentioned, certain chemicals were used, which chemicals are also used in the present process, but in addition thereto is another element which greatly facilitates the hardening of the metals, and is acted on by the other ingredients in such a manner as to produce a much better article than can be produced by following out the process set forth in the patent cited.

The scope of usefulness of many of the metals and alloys is limited by reason of the fact that in their natural state they are not completely adapted to the conditions under which it would be desirable to use them. For example it is recognized that any increased hardness in the softer forms of iron and steel would widen the scope of their usefulness, provided none of their present valuable properties, such as conductivity, be substantially deteriorated.

My invention is a composition of matter for improving certain of the physical properties of iron or steel and their alloys, without deteriorating any of the valuable properties which they may already possess, and it is primarily designed for the hardening of iron, so as to permit it to be used in cases where extreme rigidity and strength is required.

In detail my process is as follows: The metal or alloy in any of its manufactured forms is heated to a suitable temperature and immediately subjected to the action of a properly proportioned mixture of the following substances, to wit; boric acid, a double sulfate of aluminum and cyanid of potassium. In place of this I may use boric

acid, a single sulfate of aluminum and potassium cyanid. Another very efficient mixture is simply sulfate of aluminum (either the single or double sulfate) and cyanid of potassium. When a double sulfate is used, I prefer an impure form, *i. e.*, one that contains from 7½% to 15% or over of aluminum oxid. A sufficient quantity of either of these compounds is used to thoroughly cover the surface of the metal. The proportions of the ingredients may vary in accordance with the metal to be treated. A formula for general use might be cyanid of potassium one part, boric acid one part, and sulfate of aluminum one-half part. The metal or alloy thus heated is maintained at a suitable temperature (from sixteen to eighteen hundred degrees F., or higher depending upon the metal to be treated) for a sufficient length of time after which it is passed through a water solution of citric acid and aluminum sulfate, together with a salt of copper, such as the sulfate. After this the metal or alloy is cleaned and allowed to cool gradually.

The proportions of the chemical agents employed vary according to the material to be treated. The temperature at which the operations are conducted may also vary, but in the case of copper, it is about 900° F., and of brass about 1200° F.

For the purpose of carrying out the foregoing details any suitable form of furnace may be used, providing for a continuous or intermittent operation, but it is preferable that the source of heat be an impinging non-luminous flame. The aforesaid mixture of boric acid, sulfate of aluminum, and potassium cyanid, or of sulfate of aluminum and potassium cyanid may be used upon metals, especially copper and copper alloys, while in process of manufacturing into wire and other articles with gratifying results. The product is hardened or strengthened to the required degree without the admixture of alloy or without adding any alloy subsequently. Care, however, must be taken to apply the mixture in suitable quantities, and the proper heat or temperature of the metal must be ascertained by experiment. While the passage of the treated metal through the solution above mentioned is preferable, in some cases, it is a subsidiary step, and may be, in some cases, omitted.

I claim:

1. The herein described composition of matter for hardening and toughening iron and steel and their alloys, consisting of boric acid, sulfate of aluminum and potassium cyanid.
2. The herein described composition of matter for hardening and toughening iron

and steel and their alloys, consisting of one part of potassium cyanid, one part of boric acid, and one half part of sulfate of aluminum.

DAVID LAMON.

Witnesses:

FRANK B. DAVENPORT,  
WILLIAM L. INPPENLATZ.